

## UNITED STATES PATENT OFFICE.

J BIRCHARD GREEN, OF CHICAGO, ILLINOIS, ASSIGNOR TO CHICAGO STEEL & WIRE COMPANY, OF CHICAGO, ILLINOIS, A CORPORATION OF ILLINOIS.

## STITCHING WIRE.

No Drawing.

Application filed January 20, 1927. Serial No. 162,419.

My invention relates to steel wire for stitching and more particularly to flat wires for stitching cardboard boxes, fiber containers, and the like. It is desirable to have this wire quite stiff but this stiffness must be produced by cold work on comparatively low carbon steels and not through higher carbon or other alloy content. The stiffer the wire the greater thickness of stock it will 10 puncture. The higher the carbon content the quicker the cutter knives in the stitching machine will dull, and only slight dullness is required to leave a burr on the puncturing end of the legs of the stitch or staple 15 thus seriously interfering with driving it through the stock. In addition to these requirements, at least the outside fibers of the stitching wire must be sufficiently ductile to permit the clinching of the stitch without 20 cracking the wire.

These several requirements have been met in the past by using what is known as a rimmed steel of about .08% carbon content, cold-drawing it as a round wire according 25 to well-known wire-mill practice to give the correct temper and then flattening it by cold rolling to about .103" width and a variety of thicknesses from .023" to .017" inclusive and occasionally as light as .088" such as 30 will permit satisfactorily stitching in the range of work met with in practice.

The wire must be flat because it is considered desirable that the wire stitch lay practically flush with the surface of the stock. 35 A round wire would protrude substantially above this surface unless buried in the stock by force and such action would result in weakening the material at the point of stitching thus reducing the carrying capacity 40 of the box or container.

A characteristic of rimmed steel is the form of the carbide, which is essentially pearlitic in the center portion and globular in the outer or rim portion. Carbon steels 45 in which the carbide is in globular form take temper very little with cold work, while those with the carbide in pearlitic form take temper to a marked degree with cold work. The mashing flat of a round wire by cold 50 rolling appears to have comparatively little embrittling effect until the width passes about three times the thickness from which

point it increases rapidly and at about five times becomes very pronounced. This accounts for the necessity of using rimmed steel for stitching wires approximately .103" 55 in width and .023" or less in thickness. It permits producing a wire with a stiff center and a ductile shell or surface. If a steel essentially pearlitic were employed, it is 60 commercially impossible to produce the desired stiffness and surface ductility at the same time. Either can be produced alone but not both coincidentally.

The wire characteristics and proportion 65 above described have always been recognized in the industry as the fixed standards for wire used for stitching card board boxes, fiber containers, and the like.

I have discovered that by combining the 70 use of low carbon steel of .20 points or less carbon, the resultant carbide being essentially in pearlitic form, with wire dimensions such that the ratio of width to thickness does not substantially exceed four to 75 one nor substantially less than one and three quarters to one, that all the requirements of box stitching wire can readily be met. I find that widths from .050" to .070" are 80 satisfactory, and I prefer to use .060" as the most desirable width.

In this manner I can produce a box-stitching wire of substantially the same cross-sectional area as that heretofore in common use and consequently the same number of 85 feet per pound but with far greater puncturing power, or I can hold the puncturing power substantially the same as that of the wire heretofore in common use and, by reducing the cross-sectional area so that its 90 moment of inertia corresponds to a size heretofore in common use, produce a wire with far more lineal feet per pound.

I claim:

As an article of manufacture, a flat carbon 95 steel stitching wire, the carbide being essentially in pearlitic form, and the ratio of width to thickness not substantially exceeding three to one or substantially less than one and three-quarters to one.

In testimony whereof I have hereunto 100 subscribed my name.

J BIRCHARD GREEN.